

# United States Patent

[11] 3,619,196

72] Inventors **Masakuni Iwama;**  
Isaburo Inoue; Yutaka Takei; Toshihiko  
Yamamoto; Takayo Endo, Tokyo, all of  
Japan  
21] Appl. No. **868,579**  
22] Filed **Oct. 22, 1969.**  
45] Patented **Nov. 9, 1971**  
73] Assignee **Konishiroku Photo Industry Co., Ltd.**  
Tokyo, Japan  
32] Priority **Oct. 24, 1968**  
33] **Japan**  
31] **43/77030**

3,459,552 8/1969 Yoshida et al. .... 96/100  
3,481,741 12/1969 Yoshida et al. .... 96/100  
3,488,193 1/1970 Eynde et al. .... 96/100

*Primary Examiner*—John T. Goolkasian  
*Assistant Examiner*—George W. Moxon, II  
*Attorney*—Waters, Roditi, Schwartz and Nissen

**ABSTRACT:** A light-sensitive silver halide color-photographic emulsion, characterized by containing a cyan coupler represented by the general formula



wherein  $R_1$  is a hydrogen atom or a methyl group;  $R_2$  is a hydrogen atom or an aliphatic hydrocarbon residue having one to 16 carbon atoms;  $R_3$  is an aliphatic hydrocarbon residue having one to 18 carbon atoms;  $n$  is zero or 1; and  $X$  is a hydrogen atom, a halogen atom, or a substituted or unsubstituted phenylazo group.

54] **LIGHT-SENSITIVE COLOR-PHOTOGRAPHIC  
EMULSIONS**

6 Claims, No Drawings

52] U.S. Cl. .... **96/100,**  
96/55, 260/202, 260/471 A  
51] Int. Cl. .... **G03c 1/40**  
50] Field of Search.... **96/100**

56] **References Cited**

UNITED STATES PATENTS

|           |         |                         |        |
|-----------|---------|-------------------------|--------|
| 2,375,344 | 5/1945  | Bruylants et al. ....   | 96/100 |
| 2,474,293 | 6/1949  | Weissberger et al. .... | 96/100 |
| 2,562,528 | 7/1951  | Corner ....             | 96/100 |
| 3,418,129 | 12/1968 | Kimura et al. ....      | 96/100 |

# LIGHT-SENSITIVE COLOR-PHOTOGRAPHIC EMULSIONS

This invention relates to light-sensitive color-photographic emulsions containing novel cyan couplers which are soluble in water-immiscible high-boiling solvents.

As couplers for use in light-sensitive color-photographic emulsions, there are known the so-called Agfa type couplers which are soluble in water, and the so-called protected couplers which are soluble in water-immiscible high-boiling solvents. It is well known that dye images obtained by color-developing protected couplers contained in the emulsion layers of light-sensitive color-photographic materials have, in general, excellent stability to light, heat, humidity and chemicals for development as compared with those of the Agfa type couplers.

Heretofore, various compounds have been synthesized for use as protected couplers. Almost all of these, however, have disadvantages in that they are low in solubility for high-boiling solvents, they easily deposit in emulsions and coatings, the starting materials therefor are expensive, and the procedures for the synthesis thereof are complex which make them expensive. For example, the coupler of the formula



which is disclosed in U.S. Pat. No. 2,474,293, has excellent solubility for high-boiling solvents. This coupler, however, uses a very expensive starting material and is only difficultly purified. A coupler synthesized from a higher fatty acid or higher aliphatic amine, e.g. the coupler of the formula



which is described in Japanese Pat. Publication No. 2,839/64, shows excellent solubility, but the solubility is still insufficient. Moreover, there is used in said coupler an oleophilic component synthesized through several steps and therefore the coupler is expensive, even though starting materials employed are inexpensive.

In view of such actual circumstances as mentioned above, the present inventors have made various studies on couplers using inexpensive fatty starting materials to find that cyan couplers having the formula shown below, which are more excellent in solubility for high-boiling solvents, can be easily obtained.



wherein  $R_1$  is a hydrogen atom or a methyl group;  $R_2$  is a hydrogen atom or an aliphatic hydrocarbon residue having one to 16 carbon atoms;  $R_3$  is an aliphatic hydrocarbon residue having one to 18 carbon atoms;  $n$  is zero or 1; and  $X$  is a hydrogen atom, a halogen atom or a substituted or unsubstituted phenylazo group.

These couplers which are used in the present invention, can overcome the disadvantages of the conventional couplers by displaying the following characteristics:

1. They are easily soluble in such high-boiling solvents as dibutyl phthalate, tricresyl phosphate and *N,N*-dibutyl lauryl amide, so that the amounts of high-boiling solvents to be added to the couplers can be decreased and stable dispersions of high concentration can be obtained.
2. They are low in melting point and do not deposit in emulsions or in coatings.
3. They can be synthesized by a short process, they can be easily separated and purified, they are high in yields and are inexpensive in production costs.
4. They give dye images which have desirable spectral absorption characteristics and are fast to light, heat, humidity and chemicals.

Thus, the couplers employed in the present invention are quite useful as protected couplers.

Accordingly, light-sensitive color-photographic emulsions incorporated with the couplers of the present invention can be maintained stably without any deterioration in photographic characteristics due to deposition of the couplers.

Typical couplers employed in the present invention are set forth below, but these are mere examples and the couplers usable in the present invention are not limited only to these.

(1) N-Dodecyloxycarbonyl-methoxycarbonylmethyl-1-hydroxy-2-naphthamide



35 (2) N-[1-(ethoxycarbonyl)pentadecyloxycarbonylmethyl]-1-hydroxy-2-naphthamide



45 (3) N-[1-(1-methylheptyl)-oxycarbonyl-methoxycarbonylmethyl]-1-hydroxy-2-naphthamide



55 (4) N-[1-(dodecyloxycarbonyl)-cthoxy carbonylmethyl]-1-hydroxy-2-naphthamide



60 (5) N-[1-(butoxycarbonyl)-heptyloxycarbonylmethyl]-1-hydroxy-2-naphthamide



65 (6) N-[1-(dodecyloxycarbonyl-methoxycarbonyl)-ethyl]-1-hydroxy-2-naphthamide



(7) N-[2-(dodecyloxycarbonyl-methoxycarbonyl)-ethyl]-1-hydroxy-2-naphthamide



(8) N-dodecyloxycarbonyl-methoxycarbonylmethyl-1-hydroxy-4-chloro-2-naphthamide



(9) N-dodecyloxycarbonyl-methoxycarbonylmethyl-1-hydroxy-4-(2-acetylphenylazo)-2-naphthamide



(10) N-[1-(dodecyloxycarbonyl)-ethoxycarbonylmethyl]-1-hydroxy-4-(2-acetylphenylazo)-2-naphthamide



(11) N-[1-(butoxycarbonyl)-heptoxy carbonylmethyl]-1-hydroxy-4-(2-acetylphenylazo)-2-naphthamide



(12) N-[1-(dodecyloxycarbonyl-methoxycarbonyl)-ethyl]-1-hydroxy-4-(2-acetylphenylazo)-2-naphthamide



(13) N-[2-(dodecyloxycarbonyl-methoxycarbonyl)-ethyl]-1-hydroxy-4-(2-ethoxycarbonylphenylazo)-2-naphthamide

Chemical structure 9: N-[2-(dodecyloxycarbonyl-methoxycarbonyl)-ethyl]-1-hydroxy-4-(2-ethoxycarbonylphenylazo)-2-naphthamide. It shows a naphthalene ring system with a hydroxyl group at position 1, a naphthylazo group at position 2, and a 4-(2-ethoxycarbonylphenylazo) group at position 1. The naphthylazo group is linked to a phenyl ring, which is further substituted with a dodecyloxycarbonyl-methoxycarbonyl-ethyl group (-COOCH<sub>2</sub>CH<sub>2</sub>COOCH<sub>2</sub>COOC<sub>12</sub>H<sub>25</sub>).

Chemical structure 10: N-[1-(1-methylheptyl)-oxycarbonyl-methoxycarbonylmethyl]-1-hydroxy-4-(2-ethoxycarbonylphenylazo)-2-naphthamide. It shows a naphthalene ring system with a hydroxyl group at position 1, a naphthylazo group at position 2, and a 4-(2-ethoxycarbonylphenylazo) group at position 1. The naphthylazo group is linked to a phenyl ring, which is further substituted with a 1-(1-methylheptyl)-oxycarbonyl-methoxycarbonylmethyl group (-COOCH<sub>2</sub>CH<sub>2</sub>COOCH<sub>2</sub>COOCH<sub>2</sub>CH<sub>2</sub>CH<sub>2</sub>CH<sub>2</sub>CH<sub>2</sub>CH<sub>2</sub>CH<sub>2</sub>CH<sub>3</sub>).

These couplers employed in the present invention are synthesized, in general, by a process in which an amino acid such as glycine,  $\alpha$ -alanine or  $\beta$ -alanine is condensed with a naphthoic acid derivative such as phenyl-1-hydroxy-2-naphthoate to obtain an N-(1-hydroxy-2-naphthoyl)-amino acid of the formula



wherein X, R<sub>1</sub> and as defined above, and then this intermediate is formed into a potassium salt and is reacted in dimethylformamide with an alkyl ester of an  $\alpha$ -halo-fatty acid, or said intermediate is reacted in dimethylformamide with an alkyl ester of halo-fatty acid in the presence of acidic potassium carbonate.

Synthesis of the couplers is exemplified below in detail.

Synthesis of the coupler (1)

a. 1-Hydroxy-2-naphthoylglycine

84 g. of potassium hydroxide are dissolved in a mixed solution of 200 ml. of water and 400 ml. of alcohol and further 112 g. of glycine are dissolved therein. To the resulting solution are added 164 g. of phenyl-1-hydroxy-2-naphthoate and 400 ml. of alcohol and the solution is boiled under reflux for 3 hours. The solution is poured into 3 kg. of ice water and then filtered in an ordinary manner with activated charcoal. To the filtrate are added 160 ml. of concentrated hydrochloric acid and the precipitate separated thereby is filtered with suction, washed with water and pressed. The wet precipitate is then taken up in 2 liters of alcohol and boiled under reflux to completely dissolve. The resulting solution is filtered in an ordinary manner with activated charcoal. The filtrate together with 3 liters of warmed water is allowed to stand and the resulting crystals are filtered with suction, washed with 30 percent alcohol and dried to give 140 g. of pale orange needle crystals melting at 207°-209° C.

In the analogous manner, the following are obtained:

1-Hydroxy-2-naphthoyl- $\alpha$ -alanine m.p. 188°-190° C.; granulated sugarlike crystals of pale pink  
1-Hydroxy-2-naphthoyl- $\beta$ -alanine m.p. 149°-150° C.; needle crystals of pale pink

b. Dodecyl- $\alpha$ -chloroacetate

94.5 g. of  $\alpha$ -chloroacetic acid and 186.3 g. of dodecyl alcohol are dissolved in 1.5 liters of dehydrated benzene. The solution added with 5 g. of p-toluenesulfonic acid is boiled under reflux for 2 to 3 hours and the water produced during the reaction is eliminated by azeotropic distillation with

benzene. The reaction solution is then shaken with aqueous sodium carbonate solution and the benzene layer is dehydrated and distilled under reduced pressure to remove the benzene. Distillation of the residue gives 155 g. of dodecyl- $\alpha$ -chloroacetate boiling at 187°-188° C./14 mm.Hg. This product may be used in the subsequent reaction stage even after benzene is distilled off without effecting further distillation.

In an analogous manner, the following are obtained:

1-Methyl-heptyl- $\alpha$ -chloroacetate b.p. 120°-123° C./13 mm.Hg.

Dodecyl- $\alpha$ -bromopropionate b.p. (decomp.); used without distillation

Butyl- $\alpha$ -bromo caproate used without distillation

c) N-Dodecyloxycarbonyl-methoxycarbonylmethyl-1-hydroxy-2-naphthamide

123 g. Of 1-hydroxy-2-naphthoylglycine are dissolved in 600 ml. of methanol and mixed with a solution of 56 g. of potassium hydroxide in 600 ml. of methanol. Methanol is distilled off under reduced pressure. The residue is added with 1 liter of dimethylformamide and 131 g. of dodecyl- $\alpha$ -chloroacetate and the mixture is heated with stirring for 2 hours at a bath temperature of 95°-100° C. After standing to cool, the reaction mixture is poured into 10 liters of water and the separated precipitate is filtered with suction, washed with water and dried. Recrystallization from 1.5 liters of methanol gives 200 g. of the product and further recrystallization from 5 liters of n-hexane gives 170 g. of flake crystals of pale pink.

In an analogous manner, the afore-said couplers (2)-(7) are obtained. Synthesis of the coupler (8)

188 g. Of the coupler (1), N-dodecyloxycarbonyl-methoxycarbonylmethyl-1-hydroxy-2-naphthamide, are dissolved in 500 ml. of chloroform. The resulting solution is cooled to below 0° C. and mixed with a mixed solution of 66 g. of sulfonyl chloride and 200 ml. of chloroform. The solution is then allowed to stand at room temperature for 1 hour and solvent is removed by the distillation under reduced pressure. The residue is mixed with 1 liter of n-hexane and allowed to stand. The separated precipitate is filtered with suction, washed with n-hexane and dried to give 13 g. of N-dodecyloxycarbonyl-methoxycarbonylmethyl-1-hydroxy-4-chloro-2-naphthamide. Recrystallization from 1.3 liters of n-hexane gives 90 g. of powderly crystals of pale brown, melting at 69°-70° C.

Synthesis of the coupler (9)

113 g. Of o-aminoacetophenone are dissolved in diluted hydrochloric acid and diazotized with an aqueous sodium nitrite solution. The resulting solution is added to a solution of 471 g. of the coupler (1), N-dodecyloxycarbonyl-methoxycarbonylmethyl-1-hydroxy-2-naphthamide in a mixed solution of 4 liters of pyridine and 10 liters of acetonitrile at a temperature below 10° C. with stirring. Stirring is continued for 30 minutes at room temperature and 400 ml. of concentrated hydrochloric acid is added to the reaction solution and the separated precipitate is filtered with suction, washed with water and dried to give 550 g. of N-dodecyloxy-carbonyl-methoxycarbonylmethyl-1-hydroxy-4-(2-acetylphenylazo)-2-naphthamide. Recrystallization from ethyl acetate gives 310 g. of featherlike red crystals.

In the above process, use of the couplers (4), (5) and (6) in place of the starting coupler (1) provides the afore-said couplers (10), (11) and (12), respectively.

The couplers (13) and (14) can be obtained from diazotized ethyl o-aminobenzoate and the couplers (3) and (7), respectively.

Among the couplers employed in the present invention, those in which X is a halogen atom can be synthesized by treating a coupler, in which X is a hydrogen atom, with a halogenating agent such as sulfonyl chloride, thereby substituting the hydrogen atom with a halogen atom. Further, those in which X is a substituted or unsubstituted phenylazo group are synthesized by coupling a coupler, in which X is a hydrogen atom, with a substituted or unsubstituted aromatic diazonium compound.

Couplers of the aforesaid formula, in which R<sub>1</sub> and R<sub>2</sub> are hydrogen atoms and R<sub>3</sub> is a straight chain alkyl group, show excellent solubility for high-boiling solvents. However, they can be markedly enhanced in solubility by changing R<sub>1</sub> to a methyl group; R<sub>2</sub> to an alkyl group; R<sub>3</sub> to a branched alkyl group; or n to 1. R, can be changed by selecting, as the starting material, glycine,  $\alpha$ -alanine or  $\beta$ -alanine; R<sub>2</sub> by selecting  $\alpha$ -chloroacetic acid,  $\alpha$ -bromopropionic acid,  $\alpha$ -bromo-n-butyl acid,  $\alpha$ -bromo-i-butyl acid,  $\alpha$ -bromocaprylic acid or  $\alpha$ -bromolauric acid; R<sub>3</sub> by selecting lauryl alcohol, 2-ethylhexyl alcohol, 2-octyl alcohol or 7-ethyl-2-methyl-undecyl alcohol; and n by selecting glycine or  $\beta$ -alanine. All these starting materials are easily obtainable, commercially available products. In the preparation of intermediate also, alkyl esters of the  $\alpha$ -halo-fatty acids are obtained by reacting an  $\alpha$ -halo-fatty acid with an equimolar amount of an aliphatic alcohol and can be synthesized with such high purity and yield. Further, the reaction of this intermediate with 1-hydroxy-2-naphthoyl-amino acid can also be carried out easily as mentioned previously, and the desired product can be obtained with high purity and yield by simple isolation and purification operations.

Thus, the couplers employed in the present invention have such advantages that they can be synthesized through three and four steps, without necessitating any complex steps, from inexpensive and easily obtainable starting materials and can be greatly reduced in production costs as compared with conventional couplers.

30 Using the couplers synthesized in the above manner, light-sensitive color-photographic materials are prepared in the following manner:

For example, a cyan coupler employed in the present invention is dissolved in a high-boiling solvent having a boiling point of more than 180° C. such as tricresyl phosphate or dibutyl phthalate, either singly or, if necessary, in admixture with a low-boiling solvent such as butyl acetate or butyl propionate. This solution is mixed with an aqueous gelatine solution containing a surface active agent and is then emulsified by means of a high speed rotary mixer or a colloid mill. Then, the thus formed coupler dispersion is directly added to a silver halide photographic emulsion, which is coated onto a film base, a baryta paper or the like support, following by drying to remove a major proportion of the low-boiling solvent. Alternatively, the above-mentioned coupler dispersion is set and then extruded to noodle form, which is freed from the low-boiling solvent by water-washing or the like means. Then the noodle is added with warming to a silver halide photographic emulsion, which is then coated onto the aforesaid support, followed by drying.

55 The above-mentioned manner of incorporation of the coupler are merely illustrative and are not limitative. The amount of the coupler to be added to the silver halide photographic emulsion is preferably in the range of 10-100 g. per mole of silver halide, but is not always limited thereto. As the silver halide employed in the photographic emulsion, there may be used such silver salts as silver chloride, silver iodide or silver iodobromide. This emulsion may contain chemical sensitizers, e.g. sulfur sensitizers, natural sensitizers present in gelatine, reductive sensitizers and noble metal salts. The emulsion may further contain ordinary photographic additives such as, for example, antifoggants, stabilizers, antistain agents, antiirradiation agents, coating aids, and other high molecular additives. Furthermore, it may contain known carbocyanine dyes, merocyanine dyes, etc. as optical sensitizers.

The thus obtained light-sensitive color-photographic material is exposed to radioactive rays, X-rays, visible rays, infrared rays, etc., is developed with a color-developing solution containing a p-phenylene-diamine type developer and is then bleached and fixed to obtain a cyan dye image favorable in transparency and high in resistance to light, heat and humidity. The dye image is excellent in spectral absorption characteristics and has a maximum absorption in the vicinity of 680-690  $\mu$ . Alternatively, when a light-sensitive color-photographic material incorporated with an arylazo type cou-

pler, which itself has a reddish orange or red color as in the case of the coupler (10) exemplified previously, is exposed and is then treated according to the ordinary color development process, there are simultaneously obtained a cyan color negative image and a reddish orange to red color positive image. This positive color image serves, in printing the negative image onto a positive material, as a mask for correcting the undesirable absorptions in blue light and green light regions which are characteristic of the cyan color negative image. Preferable as couplers of this type are substituted phenylazo compounds having in the position ortho to the azo linkage, an alkoxy carbonyl group or a fatty acyl group.

Typical developing agents employed in developing the light-sensitive color-photographic materials of the present invention include sulfates, sulfites and hydrochlorides of N,N-diethyl-p-phenylenediamine, N-ethyl-N- $\beta$ -methane-sulfonamidoethyl-3-methyl-4-aminoaniline, N-ethyl-N-hydroxy-p-phenylenediamine, N-ethyl-N-hydroxy-2-methyl-p-phenylenediamine and N,N-diethyl-2-methyl-p-phenylenediamine.

The present invention is illustrated in further detail below with reference to examples, but it is needless to say that the examples are merely illustrative and the invention is not limited thereto.

#### EXAMPLE 1

20 g. of the previously exemplified coupler (1) were added to a mixed liquid comprising 20 ml. of dibutyl phthalate and 60 ml. of butyl acetate, and the mixture was completely dissolved at 80° C. This solution was mixed with 10 ml. of a 10 percent aqueous solution of Alkanol B (alkyl naphthalene sulfonate produced by Du Pont) and 200 ml. of a 5 percent aqueous gelatine solution, and the mixture was subjected to a colloid mill to form a coupler dispersion. This coupler dispersion was added to 1 kg. of a high speed gelatinous silver iodobromide emulsion, which was then coated onto a film base and was dried to prepare a light-sensitive color-photographic material having a stable coating layer.

The thus prepared light-sensitive material was exposed according to an ordinary procedure and was then developed at 20° C. for 10 minutes with a developing solution of the following composition:

|                                              |          |
|----------------------------------------------|----------|
| N,N-Diethyl-p-phenylenediamine hydrochloride | 2.5 g.   |
| Anhydrous sodium sulfite                     | 2.0 g.   |
| Sodium carbonate (monohydrate)               | 82.0 g.  |
| Potassium bromide                            | 2.0 g.   |
| Water to make                                | 1000 ml. |

Subsequently, the developed material was subjected to ordinary stopping and fixing treatments, was washed with water for 10-15 minutes and was then treated for 5 minutes with a bleaching bath of the following composition:

|                        |          |
|------------------------|----------|
| Potassium ferricyanide | 100 g.   |
| Potassium bromide      | 50 g.    |
| Water to make          | 1000 ml. |

The bleached material was further washed with water for 5 minutes and was then fixed for 5 minutes with a fixing bath having the following composition:

|                                   |          |
|-----------------------------------|----------|
| Sodium thiosulfate (pentahydrate) | 250 g.   |
| Water to make                     | 1000 ml. |

Thereafter, the fixed material was washed with water for 20-25 minutes and was then dried to obtain a brilliant cyan dye image having a maximum absorption at 685 m $\mu$ .

#### EXAMPLE 2

10 g. of the exemplified coupler (8) were added to a mixed liquid comprising 10 ml. of tricresyl phosphate and 30 ml. of butyl acetate, and the mixture was completely dissolved at 60° C. This solution was mixed with 5 ml. of a 10 percent aqueous

solution of Alkanol B and 200 ml. of a 5 percent aqueous gelatine solution, and the mixture was subjected to a colloid mill to form a coupler dispersion. This dispersion was added to 500 g. of a gelatinous silver iodobromide emulsion, which was then coated onto a film base and was dried to prepare a light-sensitive color-photographic material, which was free of any deposition of the coupler.

The thus prepared light-sensitive material was exposed and was then developed at 20° C. for 10 minutes with a developing solution of the following composition:

|                            |          |
|----------------------------|----------|
| Methol                     | 3.0 g.   |
| Anhydrous sodium sulfite   | 60.0 g.  |
| Hydroquinone               | 6.0 g.   |
| Anhydrous sodium carbonate | 50.0 g.  |
| Potassium bromide          | 1.0 g.   |
| Water to make              | 1000 ml. |

Subsequently, the developed material was subjected to ordinary stopping and film-hardening treatments and to water-washing. After subjecting it to second exposure by means of a white light, the material was developed at 20° C. for 12 minutes with a developing solution of the following composition:

|                                              |          |
|----------------------------------------------|----------|
| N,N-Diethyl-p-phenylenediamine hydrochloride | 5.0 g.   |
| Anhydrous sodium sulfite                     | 2.0 g.   |
| Sodium carbonate (monohydrate)               | 82.0 g.  |
| Potassium bromide                            | 1.0 g.   |
| Water to make                                | 1000 ml. |

Thereafter, the material was subjected to ordinary stopping, fixing, water-washing and bleaching treatments, was washed with running water for 20 minutes and was then dried to obtain a brilliant cyan color positive image having a maximum absorption at 685 m $\mu$ .

#### EXAMPLE 3

10.0 g. of the exemplified coupler (4) were mixed with 20 ml. of dibutyl phthalate, and the mixture was completely dissolved at 50° C. This solution was mixed with 5 ml. of a 10 percent aqueous solution of Alkanol B and 200 ml. of a 5 percent aqueous gelatine solution, and the mixture was passed several times through a colloid mill to form a dispersion. The dispersion was added to 500 g. of a gelatinous silver chlorobromide emulsion, which was then coated onto a baryta paper and was dried to prepare a light-sensitive color-photographic material.

The thus prepared light-sensitive material was exposed and then developed at 20° C. for 10 minutes with a developing solution of the following composition:

|                                                   |          |
|---------------------------------------------------|----------|
| N-Ethyl-N-hydroxyethyl-p-phenylenediamine sulfate | 2.5 g.   |
| Anhydrous sodium sulfite                          | 2.0 g.   |
| Hydroxyamine hydrochloride                        | 1.0 g.   |
| Sodium carbonate (monohydrate)                    | 82.0 g.  |
| Potassium bromide                                 | 2.0 g.   |
| Water to make                                     | 1000 ml. |

Subsequently, the material was dipped in a stopping bath comprising 10 ml. of glacial acetic acid, 3.0 g. of caustic soda and 1000 ml. of water, and was then immediately dipped for 4 minutes in an acidic, film-hardening fixing bath. Subsequently, the material was washed with water for 10 minutes and was bleached at 20° C. for 8 minutes in a bath of the following composition:

|                                                             |          |
|-------------------------------------------------------------|----------|
| EDTA 2Na (disodium salt of ethylenediamine tetracetic acid) | 40.0 g.  |
| Ferric chloride                                             | 30.0 g.  |
| Sodium carbonate (monohydrate)                              | 20.0 g.  |
| Potassium bromide                                           | 30.0 g.  |
| Sodium thiosulfate (pentahydrate)                           | 200.0 g. |
| Water to make                                               | 1000 ml. |

After washing with water for 20 minutes, the bleached material was dipped in a stabilizing bath for 2 minutes and

then dried to obtain a cyan color image having a maximum absorption at 685 m $\mu$  which was favorable in resistance to light and heat and was excellent in stability.

## EXAMPLE 4

2.0 g. of the exemplified coupler (10) were added to a mixed liquid comprising 2 ml. of dibutyl phthalate and 6 ml. of butyl acetate, and the mixture was dissolved at 80° C. This solution was mixed with 1 ml. of a 10 percent aqueous solution of Alkanol B and 20 ml. of a 5 percent aqueous gelatine solution, and the mixture was subjected to a colloid mill to form a coupler dispersion. The coupler dispersion was added to 100 g. of a high speed gelatinous silver iodobromide emulsion, which was then coated onto a film base and dried to prepare a high-sensitive color-photographic material.

The thus prepared light-sensitive material was exposed according to an ordinary procedure and was then treated with the same developing solution as in example 1 to obtain a red positive image having a maximum absorption at 500 m $\mu$  and a cyan color image having a maximum absorption at 685 m $\mu$ .

## EXAMPLE 5

2.0 g. of the exemplified coupler (7) were dissolved in 5 ml. of butyl acetate. This solution was mixed with 1.5 ml. of a 10 percent aqueous solution of Alkanol B and 20 ml. of a 5 percent aqueous gelatine solution, and the mixture was subjected to a colloid mill to form a coupler dispersion. The coupler dispersion was added to 100 g. of a red color-sensitive, high speed gelatinous silver iodobromide emulsion, which was then coated onto a film base and dried to prepare a light-sensitive color-photographic material. The thus prepared light-sensitive material was exposed according to an ordinary procedure and was then developed with the same developing solution as in example 1 to obtain a brilliant cyan color image having a maximum absorption at 685 m $\mu$ .

## EXAMPLE 6

5.0 g. of the exemplified coupler (2) were added to a mixed liquid comprising 5.0 ml. of dibutyl phthalate and 15 ml. of butyl acetate, and the mixture was dissolved at 60° C. This solution was mixed with 2.5 ml. of a 10 percent aqueous solution of Alkanol B and 50 ml. of a 5 percent aqueous gelatine solution, and the mixture was subjected to a colloid mill to form a coupler dispersion. The coupler dispersion was added to 500 g. of a red sensitized silver chloride emulsion, which was then coated onto a film base and dried.

On the other hand, 5.0 g. of  $\alpha$ -[3-(2,4-di-tert-amyl-phenoxacetamide)-benzoyl]-2-methoxy-acetanilide were dissolved and mixed with a gelatine solution in the same manner as above to form a dispersion. The dispersion was added to 500 g. of a silver bromide emulsion, which was then coated onto the above-mentioned coating to prepare a light-sensitive color-photographic material.

The thus prepared light-sensitive material was exposed to X-rays according to an ordinary procedure, was developed at 20° C. for 10 minutes with the same developing solution as in example 1, and was subjected to ordinary stopping and film-hardening treatments and to water-washing. After subjecting to second exposure by means of a yellow light (using Agfa color Separation Filter L<sub>4</sub>; exposure time 30 seconds), the material was again developed at 20° C. for 10 minutes with the above-mentioned developing solution, was subjected to ordinary stopping, fixing, bleaching and water-washing treatments, and was then dried to obtain a yellow color image with a blue background.

## EXAMPLE 7

5.0 g. of the exemplified coupler (5) were added to a mixed liquid comprising 5.0 ml. of dibutyl phthalate and 15 ml. of butyl acetate, and the mixture was completely dissolved by heating to 60° C. This solution was mixed with 2.5 ml. of a 10 percent aqueous solution of Alkanol B and 50 ml. of a 5 percent aqueous gelatine solution, and the mixture was subjected

70  
75

## 10

to a colloid mill to form a coupler dispersion. The coupler dispersion was added to 500 g. of a high speed silver iodobromide emulsion, which was then coated onto a film base and dried to prepare a light-sensitive color-photographic material.

- 5 On the other hand, a gelatine layer having a thickness of about 5  $\mu$  was formed on a cellulose triacetate film base. Onto said gelatine layer was spotted a thymidine solution, which had been labeled with tritium so that the amount thereof corresponded to 10  $\mu$ c. per cm<sup>2</sup>. Thereafter, spotting was repeated by doubling diluting of the said solution to form a standard radioactive source with a stepwedge of  $\sqrt{2}$  with respect to radioactivity.

The surface of this gelatine film was brought in close contact with the film surface of the above-mentioned light-sensitive color-photographic material. After allowing it to stand for 15 hours, the light-sensitive material was subjected to the same development as in example 1 to obtain a brilliant cyan dye image showing the presence of radioactive substance at the portion corresponding to the radioactive source.

What we claim is:

1. A light-sensitive silver halide color-photographic emulsion, comprising a cyan coupler represented by the general formula



wherein R<sub>1</sub> is a hydrogen atom or a methyl group; R<sub>2</sub> is a hydrogen atom or an aliphatic hydrocarbon residue having one to 16 carbon atoms; R<sub>3</sub> is an aliphatic hydrocarbon residue having one to 18 carbon atoms; n is zero or 1; and X is a hydrogen atom, a halogen atom, or a substituted or unsubstituted phenylazo group.

- 35 40 2. A light-sensitive silver halide color-photographic emulsion as claimed in claim 1, in which said cyan coupler is N-[1-(Dodecyloxycarbonyl-methoxycarbonyl)-ethyl]-1-hydroxy-2-naphthamide of the formula



3. A light-sensitive silver halide color-photographic emulsion as claimed in claim 1, in which said cyan coupler is N-[2(Dodecyloxycarbonyl-methoxycarbonyl)-ethyl]-1-hydroxy-2-naphthamide of the formula



4. A light-sensitive silver halide color-photographic emulsion as claimed in claim 1, in which said cyan coupler is N-Dodecyloxycarbonyl-methoxycarbonylmethyl-1-hydroxy-4-chloro-2-naphthamide of the formula



11

5. A light-sensitive silver halide color-photographic emulsion as claimed in claim 1, in which said cyan coupler is N-[1-(Dodecyloxycarbonyl-methoxycarbonyl)-ethyl]-1-hydroxy-4-(2-acetylphenylazo-2-naphthamide of the formula



5

10

15

20

25

30

35

40

45

50

55

60

65

70

12

6. A light-sensitive silver halide color-photographic emulsion as claimed in claim 1, in which said cyan coupler is N-[2-(Dodecyloxycarbonyl-methoxycarbonyl)-ethyl]-1-hydroxy-4-(2-ethoxycarbonylphenylazo)-2-naphthamide of the formula



\* \* \* \* \*